

1

2,892,776

## LUBRICATING GREASE THICKENED WITH ULTRAMARINE BLUE

Joseph F. Lyons, Wappingers Falls, and Norman R. Odell, Fishkill, N.Y., assignors to Texaco Inc., a corporation of Delaware

No Drawing. Application August 13, 1957  
Serial No. 677,823

5 Claims. (Cl. 252—28)

This invention relates to lubricating greases thickened with ultramarine blue in finely divided form.

Ultramarine blue is a double silicate of aluminum and alkali metal containing chemically combined sulfur, which is produced commercially by heating together clay, sodium carbonate and/or sodium sulfate, sulfur and a carbonaceous material such as charcoal, pitch or rosin, either with or without added silica, at temperatures of about 1500° F. for twenty-four hours or longer. It ordinarily comprises about 35 to about 50 percent by weight of silica, about 20 to about 32 percent by weight of alumina, about 18 to about 23 percent by weight of alkali metal oxide, and at least about 1 percent by weight of sulfur. The preferred materials of this character for use in accordance with the present invention are those containing about 6 to about 14 percent by weight of sulfur.

We have found that lubricating greases of improved extreme pressure properties and other advantages are obtained by dispersing finely divided ultramarine blue in lubricating oils in suitable proportions. The extreme pressure properties of these greases are substantially in excess of those obtained with other non-organic solid thickeners which have been employed as grease thickening agents heretofore, and are apparently due to the sulfur which the ultramarine blue contains.

The lubricating greases of this invention comprise an oleaginous liquid vehicle and a grease forming proportion of ultramarine blue in finely divided form, suitably in the form of particles below about 5.0 microns in diameter, and preferably from about 0.05 to about 3.0 microns in diameter. The amount of ultramarine blue employed will usually range from about 5 percent to about 45 percent by weight of the grease, and very advantageously from about 10 percent to about 40 percent by weight of the grease.

The oleaginous liquid vehicle employed in these greases may be any oleaginous liquid suitable for use in grease making generally, such as mineral lubricating oils obtained by any of the conventional refining processes, preferably refined mineral oils in the viscosity range from about 100 to 600 seconds Saybolt Universal at 100° F. Other oleaginous materials which may be used are vegetable oils such as corn oil, cottonseed oil, castor oil, etc., and animal oils such as lard oil, sperm oil, etc. For some purposes, as for preparing greases for high temperature operations, various synthetic oils may be employed with particular advantage, such as, for example, polyalkylene glycols, various high molecular weight esters and ethers, and silicone polymer oils.

The lubricating greases are prepared without the necessity for any special equipment by merely mixing together the oleaginous liquid vehicle and the ultramarine blue in finely divided form, employing any convenient means for obtaining a uniform dispersion of the solid thickener in the oleaginous liquid. A colloid mill or a mill of the type employed to grind paint pigments may be employed very advantageously for this purpose. The mixing may

2

be carried out at ordinary temperatures or somewhat higher temperatures, up to about 300° F., may be employed if desired in order to dissolve any additives employed.

5 As an example of the compositions of this invention, a grease was prepared comprising 30 percent by weight of ultramarine blue in a refined naphthene base distillate oil having a Saybolt Universal viscosity at 100° F. of about 300 seconds. The ultramarine blue was a commercial product comprising by analysis 15.8 percent by weight of sodium oxide, 26.6 percent by weight of alumina, 37.7 percent by weight of silica, 11.3 percent by weight of sulfur and 8.1 percent by weight of volatile material, or corresponding approximately to the formula  $Na_3Al_3Si_3—4S_2O_{13}$ . It was employed in the form of particles having a particle size mostly within the range 0.1-0.5, microns diameter with a minor proportion of larger particles having diameters up to about 3.0 microns, and having a measured surface area of 20 square meters per gram. The grease was prepared by stirring the two ingredients together and passing the mixture through a Premier Colloid Mill with two passes at 0.002 inch clearance. A soft blue grease of excellent texture and appearance was obtained having the following properties:

15 25 Dropping point, °F. 500+  
A.S.T.M. Working Stability Test:  
A.S.T.M. Penetration at 77° F.—  
Worked 60 strokes 343  
Worked 100,000 strokes 360

30 A.S.T.M. Bomb Oxidation Test, 100 hrs. at 210° F.:  
Pressure drop, lbs. 6

As shown by the data given above, the grease representative of the greases of this invention had a high dropping point, good shear stability and high oxidation resistance without the use of inhibitors. Table I below shows the extreme pressure properties of a grease of the composition described above in comparison with those of a grease of approximately the same grade obtained by employing 35 finely divided silica as the thickening agent in a mineral lubricating oil of the same type.

Table I

|    | Grease No.                          | 1      | 2                 |
|----|-------------------------------------|--------|-------------------|
| 45 | Thickening Agent                    | Silica | Ultramarine Blue. |
|    | Mean Hertz Load, Seizure load, Kg.  | 29     | 36                |
|    | Four Ball Navy Wear, Microns/minute | 13.2   | 9.4               |
|    | Timken, O.K. Test, lbs.             | 114    | 20                |

50 1 Obtained upon a grease of approximately the same grade prepared from a different mineral oil.

The above tests are well known laboratory tests for determining the extreme pressure and antiwear properties of lubricants. The Mean Hertz Load and Navy Wear tests are carried out as described, for example, in U.S. 2,600,056, column 12, lines 13-60, employing a test machine which comprises four steel balls in a pyramid arrangement and lubricated at their points of contact with the lubricant under test. The test comprises rotating the upper ball at a high speed in contact with the other three balls, while a load is applied to the system by means of a lever arm. The Mean Hertz Load is the load upon the lever which causes welding after 10 seconds of operation. The Navy Wear values represent the average diameter of the score marks upon the balls after one minute with a weight of 10 kilograms upon the lever arm. The Timken OK test is carried out employing the test machine described in U.S. 1,990,771. It consists essentially in rotating a flat steel ring against a steel test block wire while the area of contact is lubricated with the lubricant under test, and applying increasing loads by

five pound increments until welding occurs. The load just before the load which causes welding is the OK load.

As shown by the data in Table I, both the extreme pressure and antiwear properties of the ultramarine blue thickened grease were considerably superior to those of the silica thickened grease, which are typical of the results which have been obtained heretofore by employing inorganic solids as thickening agents in greases. The extreme pressure properties of the ultramarine blue thickened grease were also much superior to those of the conventional soap thickened greases, which ordinarily have Mean Hertz loads in about the range 20 to 25 and Timken OK values of about 10.

In addition to the ultramarine blue thickener, the greases of this invention may contain the conventional fatty acid soaps as additional thickening agents. For example, about 5 to 15 percent by weight of ultramarine blue may be added very advantageously to a grease containing about 10 to 30 percent by weight of a sodium, calcium, aluminum, or mixed base soap of stearic acid or other long chain fatty acid or hydroxy fatty acid. A superior block grease is obtained by mixing about 10 to 15 percent by weight of this material with a grease containing about 20 to 25 percent by weight of a sodium or mixed sodium-calcium soap in a heavy or residual type mineral lubricating oil.

Additives of the usual type employed in lubricating greases, such as oxidation inhibitors, corrosion inhibitors and tackiness agents, such as various high polymer materials, extreme pressure agents, etc. may also be present. As examples of particularly suitable corrosion or rust inhibitors may be mentioned metal salts of wax benzene sulfonates, metal salts of petroleum sulfonate, lauryl phosphate, sorbitol monooleate and glycerol monostearate. Suitable oxidation inhibitors include phenyl-alpha-naphthylamine, diphenyl-para-phenylenediamine, tetramethyl-diaminodiphenylmethane and bis (2-hydroxy-3-t-butyl-5-methylphenyl) methane.

With particular advantage, a surface active agent, such as a quaternary ammonium salt of a fatty acid, a poly-glycol ether, a metal alkyl sulfate or sulfonate, etc., may be employed in these greases in order to improve their water resistance and emulsification characteristics. The surface active agent may be added in any suitable man-

ner during the preparation of the grease. Very advantageously, such a compound may be employed to treat the ultramarine blue before the latter is combined with the oleaginous liquid vehicle.

Obviously, many modifications and variations of the invention, as hereinbefore set forth, may be made without departing from the spirit and scope thereof and, therefore, only such limitations should be imposed as are indicated in the appended claims.

10 We claim:

1. A lubricating grease comprising a lubricating oil as the predominating constituent, and about 5 to 45 percent by weight, based on the weight of the grease, of ultramarine blue in finely divided form, having a particle size from about 0.05 to about 3.0 microns in diameter.

2. The composition according to claim 1, wherein the ultramarine blue consists essentially of 35 to 50 percent by weight of silica, 20 to 32 percent by weight of alumina, 18 to 23 percent by weight of alkali metal oxide and 6 to 14 percent by weight of sulfur.

3. The composition according to claim 1, wherein the ultramarine blue is a material of the approximate formula  $Na_3Al_3Si_3—4S_2O_{13}$ .

25 4. The composition according to claim 1, wherein the said lubricating oil is a mineral lubricating oil having a viscosity in the range from about 100 to 600 seconds SU at 100° F.

5. A lubricating grease consisting essentially of a major portion of a mineral lubricating oil thickened to a grease consistency by about 20 to 40 percent by weight, based on the weight of the grease, of finely divided ultramarine blue having a particle size in the range of about 0.05 to 3.0 microns.

35

#### References Cited in the file of this patent

#### UNITED STATES PATENTS

|           |                 |       |               |
|-----------|-----------------|-------|---------------|
| 1,431,079 | Acheson         | ----- | Oct. 3, 1922  |
| 2,020,539 | Dourif          | ----- | Nov. 12, 1935 |
| 2,648,633 | Peterson et al. | ----- | Aug. 11, 1953 |

#### OTHER REFERENCES

Transactions, Faraday Society, London, vol. 36 pp. 45 1007-17 (1940) Articles by Mardles.